

Nov. 10, 1925.

1,561,346

F. MILLIKEN

MANUFACTURE OF ROLLED METAL DISKS

Filed Dec. 4, 1920

Fig. 1,



Fig. 2.



WITNESSES

*Edw. Thorpe*  
*John. Kostka*

INVENTOR

*Foster Milliken*  
BY *Thommes*  
ATTORNEYS

## UNITED STATES PATENT OFFICE.

FOSTER MILLIKEN, OF LAWRENCE, NEW YORK.

## MANUFACTURE OF ROLLED METAL DISKS.

Application filed December 4, 1920. Serial No. 428,331.

*To all whom it may concern:*

Be it known that I, FOSTER MILLIKEN, a citizen of the United States, and a resident of Lawrence, in the county of Nassau and State of New York, have invented new and useful Improvements in the Manufacture of Rolled Metal Disks, of which the following is a full, clear, and exact description.

The object of the invention is to provide certain new and useful improvements in the manufacture of rolled metal disks whereby the cost of production is greatly reduced and waste of material is practically eliminated.

Another object is to render the rolled metal disk exceedingly homogeneous and uniform in texture or fiber.

Another object is to permit of running the rolling mill used for rolling the disks with less power than that required for rolling rectangular sheets or plates to be subsequently cut up into disks.

In order to produce the desired result a metal disk of approximately circular form is subjected to repeated rolling actions in a rolling mill and with the disks partly turned between successive rollings to alternately elongate and circularize the disk, decrease its thickness and increase its diameter, with the fiber rolled in different directions thereby increasing the tensile strength of the disk.

In the manufacture of rolled metal disks as heretofore practiced, it has been customary to roll the metal in a rolling mill into a rectangular or square sheet or plate and then cut or stamp disks out of the sheet or plate. This cutting or stamping operation requires an expensive machine and, at least, one attendant, thus necessarily increasing the cost of manufacture of the disk besides producing a large amount of waste or scrap amounting anywhere from 25 per cent to 50 per cent of the amount of metal rolled. With my process above outlined and presently described in detail, the cost of production is reduced and the formation of scrap, if not entirely eliminated, is, at least, reduced to a minimum.

In the drawings which form a part of this specification, Figures 1 and 2 represent diagrammatic views of the successive steps in rolling out the metal disk.

A metal disk 10, cast or otherwise produced and of approximately circular shape, is passed between a pair of rolls 11 of a suitable rolling mill whereby the disk is reduced in thickness and rolled into an elongated, approximately oval or elliptic shape, that is, the diameter A, A of the disk 10 and extending transversely to the rolls 11 is increased to form the major axis of an oval or elliptical disk, while the diameter B, B of the disk parallel to the rolls 11 remains approximately the same and forms the minor axis of the oval or elliptical disk. This elongated disk is next subjected to another rolling action between the same or another pair of rolls 11 but with the disk in quarter turn position, as shown in Figure 2, that is, with the diameter B, B disposed transversely to the rolls 11. The disk in passing through the rolls in this position is elongated in the transverse direction of the diameter B, B whereby it is rolled into circular form of a larger diameter and less thickness than the disk had originally. If necessary, the foregoing two rolling actions are repeated as many times as are necessary to roll the disk until the desired predetermined diameter and thickness is reached.

The drawings indicate direction of rolling only and applicant does not limit himself to passing the disks between the rollers once but may pass the same back and forth a number of times if desired, though ordinarily if the disk is fairly hot it will become elongated as illustrated in Figure 1 with one rolling action and resume a substantially round position when rolled in a direction at right angles to the first rolling. The elongation from one rolling may be small or comparatively great, according to the hotness of metal and according to the pressure used.

Although the two successive steps above described produce the desired result, it is not absolutely necessary to give a quarter turn to the disk between successive rolling actions as this operation can be varied and the disk but slightly and progressively turned between a correspondingly large number of rolling actions to produce the desired result. It will be seen that by the method described the original circular disk is elongated and circularized by repeated rolling actions whereby the disk produced has an increased diameter and a decreased thickness in comparison with the original disk.

It will be noticed that by rolling the disk in the manner described, the direction of the fiber or texture of the metal is changed, that is, the fiber is not solely drawn in one

direction only, as is the case in rolling out sheets passed through the rolls in the same direction during each rolling operation. Thus the fiber extends in different directions and hence the tensile strength of the finished product is greater in comparison with that of similar disks cut from rolled sheets.

When rolling sheet metal a considerable torque is produced in the rolling operation owing to the rolls taking hold of the sheet throughout the entire width thereof. In rolling out a sheet as above described the torque on the metal starts at practically nothing as the front edge of the peripheral face of the disk enters between the rolls, and the torque increases gradually until it reaches its maximum at the time the disk is half way through the rolls, and then the torque gradually decreases until the disk is completely through the rolls. Thus it takes less power to run the mill for rolling out disks than is required to roll a square or rectangular sheet of about the same area. The rolling may be done with the disk either hot or cold.

Having thus described my invention, I claim as new and desire to secure by Letters Patent:—

1. The herein described method of producing a rolled metal disk of uniform thickness throughout, which consists in subjecting the entire surface of a circular disk to a rolling action between a pair of rolls to reduce the disk and elongate it in one direction, then turning the disk and again subjecting the entire disk to a rolling action between a pair of rolls to elongate the disk in another direction. 30 35

2. The herein described method of producing a rolled metal disk of uniform thickness throughout which consists passing a cast circular disk between a pair of rollers for subjecting the disk to the rolling action of said rolls to reduce the disk and 40 45 elongate it in one direction, then giving a quarter turn to the disk and again pass it between said rollers for again subjecting the disk to rolling action of said rolls to elongate the disk in another direction. 50

3. The herein described method of producing a rolled metal disk of uniform thickness throughout which consists in casting an approximately circular disk, then rolling the disk into elongated shape, then turning the disk and again rolling it into approximately circular shape. 55

FOSTER MILLIKEN.